

Sept. 3, 1940.

P. H. DOWLING

2,213,389

MANUFACTURE OF ELECTRICAL RECTIFIERS

Filed March 19, 1938



Fig. 1.



Fig. 2.



Fig. 3.



Fig. 4.

INVENTOR  
Philip H. Dowling.  
BY  
A. L. Vencill  
HIS ATTORNEY

## UNITED STATES PATENT OFFICE

2,213,389

MANUFACTURE OF ELECTRICAL  
RECTIFIERS

Philip H. Dowling, Forest Hills, Pa., assignor to  
The Union Switch & Signal Company, Swiss-  
vale, Pa., a corporation of Pennsylvania

Application March 19, 1938, Serial No. 196,911

19 Claims. (Cl. 175—366)

My invention relates to the manufacture of electrical rectifiers, and particularly to the manufacture of rectifier elements for copper oxide rectifiers.

5 One object of my invention is to improve the rectifying characteristics of the rectifier elements.

Other objects and characteristic features of my invention will appear as the description proceeds.

10 I shall describe one process of manufacture embodying my invention, and shall then point out the novel features thereof in claims.

In the accompanying drawing, Fig. 1 is a view 15 showing in elevation one form of blank ready to be prepared as a rectifier element in accordance with one process of manufacture embodying my invention. Fig. 2 is a view showing a number of blanks assembled on a support as they appear 20 during one step in the process of manufacture. Fig. 3 is a vertical sectional view showing, in an exaggerated form, a rectifier element as it appears in another step in the process of manufacture embodying my invention. Fig. 4 is a 25 view showing a completed rectifier element, constructed in accordance with my invention.

Similar reference characters refer to similar parts in all four views.

In the process of manufacturing copper oxide 30 rectifier elements, as it is now generally practiced, a number of copper blanks which may, for example, be similar to the blank A shown in Fig. 1 are first cleaned, usually by subjecting them to the action of a strong solvent for copper, and then 35 rinsing them in running tap water, that is, in water drawn from the city mains or other usual water supply. Any suitable solvent may be used, but a 50 per cent solution by volume of chemically pure nitric acid has been found to be particularly effective for this purpose. When a 50 per 40 cent solution is used, the blanks should preferably be immersed for at least 30 seconds. The blanks are then assembled in pairs on a suitable support or rack B in the manner 45 shown in Fig. 2 so that the blanks of each pair have their adjacent faces A<sup>1</sup> in contact. The blanks are then heated in the presence of air in an electric furnace, the temperature of which is usually maintained at about 1860° F. 50 This heating of the blanks causes a layer of red or cuprous oxide to be formed on the blanks, and is continued until the cuprous oxide layer is of the desired thickness. After a sufficient amount of oxide has been formed on the copper blanks, these 55 blanks are then transferred immediately to a

second furnace which is maintained at a temperature of approximately 1050° F., and are allowed to remain in this latter furnace for at least a sufficient length of time to permit them to cool down to the temperature of the second furnace. 5 The oxidized blanks are then removed from the second furnace and are suddenly cooled or quenched by plunging the blanks into cold water. Each blank then appears as shown in Fig. 3, from which it will be seen that each blank A is now 10 covered with an inner coating D of cuprous or red oxide of copper and a thin outer coating C of black oxide of copper. It will also be seen from an inspection of Fig. 3 that the flat face of the blank which is exposed during the oxidizing 15 process, that is to say, the lower face has a much heavier oxide coating than the upper face. Each blank is next treated to remove the black oxide from the lower face of the blank, and both the black and red oxide from the upper face, after 20 which the blank will appear as shown in Fig. 4. One process which is particularly suitable for removing the excess oxide from the blanks is described and claimed in Letters Patent of the United States No. 2,094,642, granted to me on 25 October 5, 1937. As a last step, the electrical contact to the exposed face of the cuprous oxide remaining on the blanks is improved as by rubbing into this face powdered petroleum coke.

Rectifier elements of the type described exhibit 30 the characteristic of offering a relatively low resistance to current flowing through the elements from the cuprous oxide to the copper and a relatively high resistance to the flow of current through the elements in the opposite direction. 35 The resistance of the elements in the low resistance direction will hereinafter be referred to as the conducting resistance, while the resistance of the elements in the high resistance direction will hereinafter be referred to as the blocking resistance. 40

Rectifier elements of the type described also exhibit the characteristic that when a voltage is applied to them in the high resistance or blocking direction, the high or blocking resistance will decrease at first relatively rapidly and then somewhat more slowly with time until it attains an apparently stable value which may be considerably less than the initial value. The stable virtual value of the reverse current when an alternating 50 voltage is applied to the rectifier is increased due to this effect, and this effect accordingly in some instances determines the voltage for which the rectifier is capable of effecting satisfactory rectification in service. This change in blocking re- 55

- sistance with time is ordinarily known as "creep," or "reverse creep," and is usually temporary in character, the apparent resistance in the reverse direction gradually returning toward its original 5 value when the voltage is removed.
- Rectifier elements of the type described further exhibit the characteristic that as time goes on the resistance of the rectifier in the low resistance or conducting direction gradually increases.
- 10 This increase in the conducting resistance with time is ordinarily known as aging, and at ordinary room temperature is quite normal. However, at elevated temperatures this aging becomes more rapid.
- 15 I have found that when rectifier elements are manufactured by the process previously described, the presence in the oxidizing furnace of certain anodic impurities has an adverse effect on the initial resistance in the blocking direction 20 of the finished rectifiers and also on the magnitude of the creep, but has a beneficial effect on the initial resistance and aging of the rectifiers in the conducting direction. These impurities may reach the oxidizing furnace from a number 25 of sources. For example, they may accumulate on the copper blanks from exposure prior to being placed in the furnace, or they may be left on the blanks by reagents or by the use of impure rinsing water in the precleaning operation, 30 or they may be present in the form of dissolved gases, or they may be introduced into the furnace on the forks or racks used to support the blanks during oxidation. In accordance with my 35 present invention, I propose to modify the previously described process by the addition of certain steps, whereby the amount and kind of impurities which are present in the oxidizing furnace can be controlled in a manner to control the effects produced by these impurities.
- 40 The first step which I have added to the hereinbefore described process to control the anodic impurities consists in washing the blanks in distilled water immediately after they have been rinsed in tap water following the acid bath, and 45 its purpose is to remove from the blanks all impurities which may be left on them following the tap water rinse. In some instances, the removal of the impurities can be facilitated by boiling the distilled water or maintaining it at the 50 boiling point. The time the blanks are left in the distilled water is not critical, but it is desirable to leave them in the water for at least 3 minutes. This step can be utilized in connection with the hereinbefore described process 55 without the addition of the other steps to be described hereinafter, and its effects in most instances appear to be to cause the elements to have a somewhat higher resistance in both directions than would otherwise be obtained, and 60 also to reduce the tendency to creep. These effects are not radical, and, while the initial resistance values in the high resistance direction will be rather uniform, the magnitude of the creep will be somewhat erratic. This erratic 65 behavior as regards creep depends to a certain extent, at least, upon small variations in the original metallic impurities which are present in the copper from which the blanks are formed, and can be eliminated and the magnitude of the 70 creep much reduced by the use of copper containing a small amount of lead as described in my copending application for Letters Patent of the United States, Serial No. 196,912, filed by me on March 19, 1938, for Electrical rectifiers.
- 75 The second additional step which may be

added to the hereinbefore described process for controlling the anodic impurities consists in treating the supports on which the blanks are mounted while they are being oxidized just prior to mounting the blanks on the supports to remove any impurities which may be present on the supports. This treatment is generally necessitated by the fact that the quenching of the blanks of each charge following their oxidation is usually effected by immersing the blanks while 10 still assembled on the supports in tap water, with the result that any impurities which may be deposited on the supports due to the presence of impurities in the tap water subsequently remain on the supports when they are next used to effect 15 the oxidation of a new charge of elements. In accordance with my present invention, these impurities are removed either by thoroughly washing the supports in distilled water, or by raising them to the temperature (or higher) at which 20 the oxidation of the blanks is to be carried out, and then allowing the supports to dry or cool in clean air, as the case may be. When the last-mentioned method of cleaning the supports is used, it is preferable to retain the supports at 25 the oxidation temperature at least as long as is normally required to oxidize the blanks.

The addition of this and the previously described step to the hereinbefore described process yields rectifiers whose initial resistances in both directions are considerably higher than those of rectifiers produced by older methods. Furthermore, the magnitude of creep is very low and very uniform, and is more or less independent of small variations in the original metallic impurities in the copper blanks. For some applications of rectifiers, the increase in the value of the resistance in the conducting direction which these additional steps produce is not desirable, but, for many other applications, a small value 4 of resistance in the conducting direction is secondary to an ability to maintain a high resistance value in the high resistance direction, and, for such applications, the hereinbefore described process modified by the addition of the two steps just described is particularly well suited.

As will readily be seen from the foregoing description, the two steps just described are calculated to remove from the blanks and racks, respectively, all impurities. The steps which I shall next describe are calculated to introduce anodic impurities into the process of manufacture in controlled amounts. Tests made with a large number of foreign materials indicate that, in general, any anion introduced into the process, or the copper, in such a way that this anion (or one of its constituent atoms) will be taken up by the copper oxide, will produce the effects mentioned hereinbefore. Some anions which have been successfully used are chlorine, carbon dioxide, iodine and the sulphate radical. However, I prefer to use either carbon dioxide or chlorine, and one way which has been found suitable to introduce these anions into the process consists in dipping the elements, or the supports on which the elements are mounted, or both, into a solution of distilled water containing carbon dioxide or chlorine following the thorough cleaning of these elements in the manner described hereinbefore. The concentration of carbon dioxide in the solution when carbon dioxide is used does not appear to be critical, and a solution saturated at atmospheric pressure is satisfactory. However, if desired, the concentration of the carbon dioxide may be increased by supersaturating the water.

or by using the water under a high carbon dioxide pressure and at a low temperature. The chlorine content of the distilled water when chlorine is used may vary between a few parts to perhaps one hundred parts per million by weight.

In special cases where creep in the high resistance direction is of no importance, or where the copper blanks have a high lead content, the chlorine might be used in greater concentration.

10 It should be mentioned that if metallic cations are introduced into the manufacturing process in such a way as to be taken up by the copper oxide, in general, the opposite effects to those produced by anions may be expected. Thus the use of a 15 salt, such as sodium chloride or sodium cyanide, produces a combination effect, and in some cases it may be desirable to use such a salt in proper concentrations.

10 If the supports on which the elements are mounted do not come into contact with any contaminating substances throughout the manufacturing process, the desired amount of impurities may be added to the supports by quenching them with their load of oxidized blanks in water containing the desired anion, thus eliminating the necessity for any special treatment of the supports.

15 It should be particularly pointed out that the steps which I have described need not necessarily all be used together, but that any combination of these steps may be employed to effect any particular desired result.

20 It should also be pointed out that the characteristics of the rectifiers obtained by the process embodying my invention can be varied to adapt the rectifier for any particular type of service by controlling the amount of the impurities introduced into the process. Furthermore, by virtue of the fact that the amount of impurities present 25 in the process are controlled, rectifiers having a high degree of uniformity are obtained.

20 It should also be pointed out that rectifiers manufactured in accordance with the process embodying my invention can be further improved 30 by employing blanks containing lead in small concentrations, and that such rectifiers are superior as regards stability in the high resistance direction to rectifiers produced in the absence, or near absence, of all impurities in or on the blanks 35 or racks or in the furnace during the oxidizing process. It should further be noted that the presence of the cathodic impurity lead in the copper sacrifices very little as regards the rectifying characteristics of the elements in the low resistance direction, at least at voltages at which the rectifiers are usually used, over what can be obtained by the incorporation into the process of a controlled amount of an anodic impurity.

35 Although I have herein shown and described only one process of manufacture of electrical rectifiers embodying my invention, it is understood that various changes and modifications may be made therein within the scope of the appended 40 claims without departing from the spirit and scope of my invention.

40 Having thus described my invention, what I claim is:

1. The process of preparing a rectifier element 45 which consists in immersing a copper blank for approximately 30 seconds in a 50 per cent solution by volume of chemically pure nitric acid, rinsing the blank in tap water to remove all traces of the acid, rinsing the blank in distilled 50 water to remove all impurities adhering to the

blank from the tap water, and then heat treating said blank to form an oxide layer thereon.

2. The process of preparing a copper oxide rectifier element from a copper blank which consists in treating the copper blank to remove all surface impurities, dipping the blank in a solution of distilled water containing carbon dioxide, and then heat treating said blank to oxidize it.

10 3. The process of preparing a copper oxide rectifier element from a copper blank which consists in treating the copper blank to remove all surface impurities, immersing the blank in a solution of distilled water which is saturated at atmospheric pressure with carbon dioxide, and then heat treating said blank to oxidize it.

15 4. The process of preparing a copper oxide rectifier element from a copper blank which consists in treating the copper blank to remove all surface impurities, subjecting the blank to a solution of distilled water containing carbon dioxide in small concentration, and then heat treating said blank to oxidize it.

20 5. The process of forming a copper oxide rectifier which consists in adding an anion to a copper body containing lead, and then heat 25 treating said body to oxidize it.

25 6. The process of preparing a copper oxide rectifier element from a copper blank which consists in treating the copper blank to remove all surface impurities, subjecting the blank to a solution of distilled water containing chlorine in small concentrations, and then heat treating 30 said blank to oxidize it.

35 7. The process of preparing a copper oxide rectifier element from a copper blank which consists in treating the copper blank to remove all surface impurities, subjecting the blank to a solution of distilled water containing a sulphate radical in small concentrations, and then heat treating said blank to oxidize it.

40 8. The process of preparing a copper oxide rectifier element from a copper blank which consists in treating the copper blank to remove all surface impurities, subjecting the blank to a solution of distilled water containing chlorine in any amount between a few parts and one hundred parts per million by weight, and then heat 45 treating said blank to oxidize it.

45 9. In the process of preparing rectifier elements from copper blanks in which the blanks are oxidized by mounting them on a support in an oxidizing atmosphere, the step which consists in baking the support at the oxidizing temperature to remove all surface impurities immediately before mounting the blanks on the 50 support.

50 10. In the process of preparing rectifier elements in which a copper blank is mounted on a support in an oxidizing atmosphere, the steps which consist in removing all impurities from the blank and the support just prior to mounting the blank on the support and subsequently adding to both the blank and the support an anion.

55 11. In the process of preparing a rectifier element from a copper blank which consists in cleaning the blank, assembling it on a support and subjecting it to an oxidizing atmosphere, and then quenching the support and blank in tap water, the step which consists in washing the support in distilled water prior to assembling the 60 blank on it to remove impurities adhering to it from a previous immersion in tap water.

65 12. In the process of preparing a rectifier element from a copper blank which consists in cleaning the blank, assembling it on a support 65

70

75

and subjecting it to an oxidizing atmosphere, and then quenching the support and blank in tap water, the step which consists in baking the support at the oxidizing temperature to remove all surface impurities immediately before mounting the blank on the support.

13. In the process of preparing a rectifier element from a copper blank which consists in cleaning the blank, assembling it on a support 10 and subjecting it to an oxidizing atmosphere, and then quenching the support and blank in tap water, the steps which consist in treating the support to remove all impurities adhering to it from a previous immersion in tap water and 15 then immersing said support in a solution containing a known amount of an anion.

14. In the process of preparing rectifier elements from copper blanks in which the blanks are oxidized by placing them on a support in an 20 oxidizing atmosphere, the steps just prior to oxidizing the blanks which consist in treating both the blanks and the supports to remove all surface impurities.

15. The process of forming a copper oxide 25 rectifier which consists in treating a copper body containing lead to remove all surface impurities, adding to the body an anion by immersing the body in a solution of distilled water containing

the anion, and then heat treating said body to oxidize it.

16. The process of forming a copper oxide rectifier which consists in immersing a copper blank containing lead in a solution of nitric acid, 5 immersing said blank in tap water to remove all traces of the acid, rinsing said blank in a solution of distilled water containing an anion, and heat treating said blank to oxidize it.

17. The process of preparing a copper oxide 10 rectifier element from a copper blank which consists in dipping the blank in a solution of distilled water containing carbon dioxide, and then heat treating said blank to oxidize it.

18. The process of preparing a copper oxide 15 rectifier element from a copper blank which consists in subjecting the blank to a solution of distilled water containing chlorine in small concentrations, and then heat treating said blank to 20 oxidize it.

19. The process of preparing a copper oxide rectifier element from a copper blank which consists in subjecting the blank to a solution of distilled water containing a sulphate radical in small concentrations, and then heat treating 25 said blank to oxidize it.

PHILIP H. DOWLING.